

A.F. & J.H. Andrews.  
Disintegrating Mach.

No. 64,058. Patented Apr. 23, 1867.

Fig: 1.



Fig: 2.



Witnesses:

D. Watson

H. C. Day

Inventor.  
Albert F. Andrews  
John H. Andrews  
By their attorney, Thomas D. Watson.

# United States Patent Office

ALBERT F. AND JOHN H. ANDREWS, OF AVON, CONNECTICUT.

*Letters Patent No. 64,058, dated April 23, 1867.*

## IMPROVED MODE OF TREATING FLAX.

The Schedale referred to in these Letters Patent and making part of the same.

TO ALL WHOM IT MAY CONCERN:

Be it known that we, ALBERT F. and JOHN H. ANDREWS, of Avon, in the county of Hartford, in the State of Connecticut, have invented certain new and useful improvements in the Treatment of Flax.

The object of our invention is to remove the glutinous matters enveloping the primary or cell fibres of flax so that they can be more readily separated from each other by picking, carding, or other suitable machinery.

We will first describe the mechanical devices which can be used to facilitate the chemical treatment. We employ a skeleton cylinder placed within a tank, which tank holds the chemical solutions, while the cylinder contains the flax and is slowly rotated during the process, the lower half of said cylinder being immersed in the different solutions while the upper half is above and out of the same. This secures a thorough circulation of the solutions used, as gravity drains off the solutions from the upper half of the cylinder, while the slow rotation of the cylinder constantly immerses the lower half of the same. The tank may be made open at the top, but a cover can be fitted at the top to exclude the air when desired. The cylinder and tank may be made of a size suitable to hold five hundred or one thousand or two thousand pounds of flax, or more or less, as may be judged best. The skeleton cylinder can be made of various materials, but wood is probably the best on account of the chemical action of alkalies and acids on the cheap metals. The cylinder is made skeleton or open-work in structure so as to admit the solutions and retain the flax. The central shaft can be made of wood, or if of iron it should be covered with vulcanized rubber or other protection to prevent its corrosion by acids. Arms can be extended from the shaft to support the main body of the cylinder. There should be a longitudinal open space in the centre of the cylinder, immediately around the shaft, of one foot or eighteen inches in diameter, as an escape for the solutions from the upper half of the cylinder. It will also answer the purpose for introducing an air-blast through the flax to dry it, and to aid in the disintegration of the fibre at the close of the process. This open space should be surrounded with longitudinal slat-work, to keep the flax in the body of the cylinder from filling it. The heads or ends of the cylinder, except this open space, may be closed with plank or boards. The outside or circumference of the cylinder may be covered with slats made of plank, two or three inches wide, with spaces between a little less than the width of the slats. The cylinder should also be divided into quarter sections of slat-work, the same as on the outside, to keep the flax in position. Two or three movable pieces can be left on each section for filling and emptying the sections.

The accompanying drawings form a part of this specification.

Figure 1 is a cross-section of the cylinder just described.

Figure 2 is a corresponding section, showing an arrangement of double net-work carrying rollers and squeezing devices.

A is the open central space in the cylinder, B B are the slatted partitions. C is the outside of the skeleton cylinder. D is the central shaft.

Another mechanical arrangement, having some advantages over the cylinder just described, is to employ a tank two or three times as long as wide, in which is placed an endless net-work in which the flax is enclosed. The twine of which the net-work is composed is covered with vulcanized rubber to prevent the action of the chemicals upon it. The net-work is double and contains the flax between the two thicknesses. It is suspended over rollers at the ends of the tank, and is carried around like an endless belt by motion given to the rollers. On the outside of the net-work other rollers, nearly in contact with those sustaining the net-work, are placed to act as pressure-rollers to press out the solutions from the flax. Other sustaining-rollers are used, in addition to those above described, to aid in sustaining the loaded net-work, to prevent sagging and undue strain on the netting. The operation of this arrangement is similar to that of the skeleton cylinder, with the advantage of being able to use pressure-rollers to press out the different solutions. It also facilitates washing the flax.

E is the interior and F the exterior portion of the double net-work. G and H are the main rollers over which it passes. I I are the sustaining-rollers. J is a pressure-roller, which is weighted or provided with springs connected with its bearings so that it may yield.

Better results can be obtained from unrotted flax than from that which has been rotted. With the cylinder or net-work loaded with the flax, cold water, or warm water below the temperature of 110° Fahrenheit, is introduced and allowed to remain ten or fifteen minutes, when it is withdrawn and fresh water introduced. Alternate cold and warm water is used until five or six changes have been made within the space of two or three hours. The warm water in the last one or two applications can be raised to 120° or 130°. After two or

three hours the warm-water process should be arrested and the flax treated to boiling water for an hour, or it should be treated with ground beans or peas in cold water, the soluble portion only being used, for a half hour, when the liquid should be withdrawn and the flax rinsed with cold water. This arresting of the process should be performed as soon as the flax shows any indication of fermentation by turning brown. The flax should next be treated with alkali. To a given quantity of caustic soda ash or carbonate of soda add twice the amount of lime. This lime in solution in a caustic state aids in dissolving the acid portion of the glutinous matter in the flax. When the alkaline solution has been introduced into the tank the temperature should be gradually raised to the boiling point. The flax should be boiled for three or four hours, after which the alkaline solution should be withdrawn and water let into the tank to wash the flax thoroughly, after which it may be steeped in a hot, weak solution of soda, or its carbonate, or a cold solution of common salt, or chloride of calcium, or muriatic acid; or any two or all three of the last-mentioned ingredients may be used together in the same solution. The use of these last-mentioned ingredients is not absolutely necessary to the successful disintegration of the fibre, but more delicate results and easier bleaching can usually be obtained by it. After washing from the above solutions the flax is ready for bleaching. To any given quantity of chloride of lime may be added an equal or less quantity of lime which has been previously neutralized with muriatic acid to change it to chloride of calcium. Water can be added to this mixture to obtain any desired degree of strength, and the length of time required in bleaching will depend on the strength and temperature of the solution. The addition of chloride of calcium or other metallic chlorides changes the chloride of lime solution from an alkaline to a neutral or, acid character, and aids in dissolving the alkaloid portion of the gluten among the fibres not soluble in alkalies.

Another mode of bleaching, whether the above solution or ordinary chloride of lime is used, is to immerse the flax in the solution and then withdraw the solution and expose the flax to atmospheric air. To facilitate the process air can be forced through the flax in the cylinder from the opening in the centre thereof. This can be done by means of a fan-blower or air-pump, and connections, which may be readily constructed by mechanics. I believe that the oxygen of the atmosphere, in the presence of chlorine, takes the active form of ozone and attacks the carbon of the gluten. Disintegration is more easily effected in this manner than by chloride alone. After bleaching the flax should be washed clean of the solution, and can then be treated with good effect by soda, or lime, or the chlorides of sodium or calcium, either separately or combined. The solutions can be used hot or cold, but the hot solution produces the best effect. The use of alkali after bleaching is not necessary, but renders the subsequent treatment easier. The flax, after being washed, should receive a weak bath of muriatic acid, diluted with water, to remove all the alkali that may remain in the flax, and should then be treated with a weak solution of urine in water, to remove all the chlorine that may be present in it, and to soften the fibre. The flax should next be treated to a weak boiling solution of soap, then rinsed, and again treated to a weak solution of urine, heated to 120° or 130°, again washed and exposed to the air for a short time, and then treated to a weak solution of cider diluted with water, after which it is ready to dry without washing out the cider solution. Warm air from 90° to 110° forced through the flax in the cylinder aids both in drying it and in its disintegration. Vinegar, beer, or any other product of fermentation, can be substituted for cider with good effect, or cider can be used instead of urine with similar results.

Having now fully described our invention, what we claim as new, and desire to secure by Letters Patent in the treatment of flax, to remove the gelatinous matters enveloping the original or cell fibres, is as follows:

1. We claim treating it by the aid of the endless double net-work, arranged relatively to the rollers G H, and to the tank, substantially as and for the purpose herein specified.
2. We claim, in connection with the above, subjecting it to the action of the pressure-roller J, arranged as represented.
3. We claim the alternate application of warm and cold water, substantially in the manner and for the purpose herein described.
4. We claim the treatment in the soluble protein solution obtained from ground beans, or other equivalent, substantially as specified.
5. We claim the treatment with the chloride of sodium, or its equivalent, after the treatment with the alkali, before the bleaching, substantially as herein specified.
6. We claim the employment of metallic chlorides in the bleaching bath, substantially as and for the purpose herein specified.
7. We claim blowing atmospheric air through the interstices after the material to be bleached has been emerged in a solution containing chloride of lime, whether this solution is prepared in the ordinary manner or as above described.
8. We claim the use of alkaline solutions after bleaching, substantially as and for the purpose herein specified.
9. We claim the treatment with urine, in connection with the treatment with soap, substantially as and for the purpose herein specified.
10. We claim the treatment with cider, or equivalent vegetable acid solution, at the termination of the process.
11. We claim the use of atmospheric air, forced through the flax, in connection with an alkaline solution, saturating the flax, as a bleaching and disintegrating agent, substantially as herein specified.

ALBERT F. ANDREWS,  
JOHN H. ANDREWS.

Witnesses:

FREDERICK RIPLEY,  
M. H. BARTLETT.